

## UNITED STATES PATENT OFFICE.

ALFRED C. DODMAN, JR., OF SUMMIT, NEW JERSEY.

## METHOD OF PREPARING WALL COVERING.

No Drawing.

Application filed September 13, 1924. Serial No. 737,627.

My present invention relates to an improvement in wall paper, and other paper and in the method of manufacture thereof, with particular relation to a method of applying to the surface of the paper coloring matter economically and with desirable decorative effects.

The object of my invention is to provide a method of applying color to paper to produce stippled effects, shaded effects, or solid color effects by means of a carrier or vehicle which is soluble or dissociated by water by sprinkling or otherwise applying the color bearing vehicle to the paper while yet in the pulp state as by sprinkling it in the powdered form onto the pulp while on the wires of a paper making machine.

Other objects of my invention will appear from the specification and claims.

In the practice of the method of my invention I combine a color of the desired shade etc., either mechanically or chemically with a carrier or vehicle which is soluble or dissociated by water and prepare a powder therefrom or otherwise reduce the combination to a finely divided state. The method of preparing the color and carrier in the finely divided state depends of course on the nature of the carrier or of the carrier when loaded with its color. Some vehicles as a sugar for example are crystallized out from solution together with the color into a granular state; others are abraded, ground, or macerated; in still other cases a heavy solution of carrier and color is sprayed into an atmosphere in which it is coagulated in hardened drops of small size. For a carrier or vehicle I use a dextrine, a glucose, a sugar, gum arabic, or any suitable water soluble agglutinant such as are well known in the art. In the addition of color according to the wet pulp it is sprinkled on in the powdered or finely divided state as by running through a rotating cylindrical screen positioned above the pulp on the wires of a paper making machine. In other cases a solution of color and vehicle are sprayed onto the screen at such a distance therefrom and under such temperature and other atmospheric conditions that the carrier will coagulate before striking the pulp. The solid particles of carrier and color will be softened by the water of the pulp with the result that they will adhere to the pulp and spread in spots or stipples which comprise a body of color held to the surface of the pulp by agglutinant. The agglutinant and color dry with the pulp when it is subjected to its drying process such as are employed and well known in the art. The amount of color added to the pulp as it passes over the wires is varied when shaded effects are desired. When solid colors are desired the particles are added in such numbers as will cover the paper to the desired shade of color. When I desire to stipple the paper with more than one color for example I apply particles of more than one color and in amounts in accordance with the relative proportions of color desired on the paper. Still other effects I obtain by mixing the color and carrier particles with other particles such as for example as particles of aluminum flake such as are described in my copending application Serial Number 737,628 filed September 12, 1924 or by otherwise applying a color and the aluminum flakes. For colors I employ any of the colors known in the art which are soluble in solvents suitable for the carrier. When I load the carrier with the color mechanically however it is only necessary that the color be suspended in the solvent while the carrier is being dissolved in the solvent. It is to be understood however that other means of mixing color and carrier and applying them are within the scope of my invention.

I claim:

1. The method of applying color to paper which comprises adding a carrier to a color, drying the carrier and color and adding the color and carrier in a finely divided state to the paper pulp while on the wires of a paper making machine.

2. The method of applying color to paper which comprises adding a water soluble carrier to a color, drying the carrier and color, reducing the resultant mass to a finely divided state, and applying the color and carrier in a finely divided state to the paper pulp while on the wires of a paper making machine.

3. The method of applying color to paper which comprises impregnating a water soluble carrier with a color or colors, rendering said carrier into a finely divided state, and sprinkling such powder onto the paper pulp on the wires of a paper making screen.

4. The method of applying color to paper which comprises sprinkling the color with

1,623,620

a water soluble carrier in a dry and finely divided state onto the paper while the paper is wet.

the paper pulp on the wires of a paper making machine.

5. The method of applying a dry color with a stippled effect to paper which comprises sprinkling color impregnated water soluble carrier in a finely divided state onto

Signed at New York in the county of New York and State of New York this 3rd day of September A. D. 1924.

ALFRED C. DODMAN JR.